



US006764366B1

(12) **United States Patent**  
Lee et al.

(10) **Patent No.:** **US 6,764,366 B1**  
(45) **Date of Patent:** **Jul. 20, 2004**

(54) **ELECTRODE STRUCTURE AND METHOD FOR FORMING ELECTRODE STRUCTURE FOR A FLAT PANEL DISPLAY**

(75) Inventors: **Jueng Gil Lee**, Cupertino, CA (US); **Christopher J. Spindt**, Menlo Park, CA (US); **Johan Knall**, Sunnyvale, CA (US); **Matthew A. Bonn**, Saratoga, CA (US); **Kishore K. Chakravorty**, San Jose, CA (US)

(73) Assignees: **Candescent Intellectual Property Services, Inc.**, Los Gatos, CA (US); **Candescent Technologies Corporation**, Los Gatos, CA (US)

(\*) Notice: Subject to any disclaimer, the term of this patent is extended or adjusted under 35 U.S.C. 154(b) by 193 days.

(21) Appl. No.: **09/999,755**

(22) Filed: **Oct. 31, 2001**

**Related U.S. Application Data**

(62) Division of application No. 09/421,781, filed on Oct. 19, 1999.

(51) **Int. Cl.** <sup>7</sup> **H01J 9/02**

(52) **U.S. Cl.** **445/24**; 445/50

(58) **Field of Search** **445/24, 50**

(56) **References Cited**

**U.S. PATENT DOCUMENTS**

4,561,009 A 12/1985 Yonezawa ..... 357/67

|              |           |                         |           |
|--------------|-----------|-------------------------|-----------|
| 4,940,916 A  | 7/1990    | Borel et al. ....       | 313/306   |
| 5,090,932 A  | * 2/1992  | Dieumegard et al. ....  | 445/21    |
| 5,191,217 A  | 3/1993    | Kane et al. ....        | 250/423 F |
| 5,283,500 A  | 2/1994    | Kochanski ....          | 315/58    |
| 5,319,279 A  | 6/1994    | Watanabe et al. ....    | 313/309   |
| 5,509,839 A  | 4/1996    | Liu ....                | 445/24    |
| 5,587,623 A  | * 12/1996 | Jones ....              | 313/309   |
| 5,594,297 A  | 1/1997    | Shen et al. ....        | 313/309   |
| 5,601,466 A  | 2/1997    | Shen et al. ....        | 445/24    |
| 5,866,979 A  | 2/1999    | Cathey, Jr. et al. .... | 313/496   |
| 5,894,188 A  | * 4/1999  | Chakravorty et al. .... | 313/309   |
| 6,019,657 A  | 2/2000    | Chakravorty et al. .... | 445/24    |
| 6,064,149 A  | 5/2000    | Raina ....              | 313/497   |
| 6,106,352 A  | 8/2000    | Fujii ....              | 445/24    |
| 6,320,138 B1 | * 11/2001 | Kamiya et al. ....      | 174/250   |

\* cited by examiner

*Primary Examiner*—Kenneth J. Ramsey

(57) **ABSTRACT**

An electrode structure for a display that includes lower electrodes and upper electrodes. In one embodiment, lower and upper electrodes are formed of either an aluminum alloy or a silver alloy. In another embodiment, upper and lower electrodes are formed using a metal alloy layer over which a cladding layer is deposited. A silicon nitride passivation layer is used to protect the upper electrodes from damage in subsequent process steps. Various other materials and structures are also disclosed that protect the upper electrodes from damage in subsequent process steps.

**38 Claims, 120 Drawing Sheets**





FIGURE 1



FIGURE 2



FIGURE 3



FIGURE 4A



FIGURE 4B



FIGURE 5A



FIGURE 5B



FIGURE 6A



FIGURE 6B



FIGURE 7A



FIGURE 7B



FIGURE 8A



FIGURE 8B



FIGURE 9A



FIGURE 9B



FIGURE 10A



FIGURE 10B



FIGURE 11A



FIGURE 11B



FIGURE 12A



FIGURE 12B



FIGURE 13A



FIGURE 13B



FIGURE 14A



FIGURE 14B



FIGURE 15



FIGURE 16A



FIGURE 16B



FIGURE 16C



FIGURE 16D



FIGURE 16E



FIGURE 16F



FIGURE 16G



FIGURE 16H



FIGURE 16I



FIGURE 16J

**FIGURE 17**



FIGURE 18A



FIGURE 18B



FIGURE 18C



FIGURE 18D



FIGURE 18E



FIGURE 18F



FIGURE 18G



FIGURE 18H



FIGURE 18I



FIGURE 18J



FIGURE 18K



FIGURE 18L



FIGURE 18M



FIGURE 18N

**FIGURE 19**



FIGURE 20A



FIGURE 20B



FIGURE 20C



FIGURE 20D



## FIGURE 20E



FIGURE 20F



FIGURE 20G



FIGURE 20H



FIGURE 20I



FIGURE 20J



FIGURE 20K



FIGURE 20L

**FIGURE 21**



FIGURE 22A



FIGURE 22B



FIGURE 22C



FIGURE 22D



FIGURE 22E



FIGURE 22F



FIGURE 22G



FIGURE 22H



FIGURE 22I



FIGURE 22J



FIGURE 22K



FIGURE 22L



FIGURE 22M



FIGURE 22N



FIGURE 23



FIGURE 24A



FIGURE 24B



FIGURE 24C



FIGURE 24D



FIGURE 24E



FIGURE 24F



FIGURE 24G



FIGURE 24H



FIGURE 241



FIGURE 24J



FIGURE 24K



FIGURE 24L



FIGURE 24M



FIGURE 24N



FIGURE 25



FIGURE 26A



FIGURE 26B



FIGURE 26C



FIGURE 26D



FIGURE 26E



FIGURE 26F



FIGURE 26G



FIGURE 26H



FIGURE 26I



FIGURE 26J



FIGURE 26K



FIGURE 26L



FIGURE 27



FIGURE 28A



FIGURE 28B



FIGURE 28C



FIGURE 28D



FIGURE 28E



FIGURE 28F



FIGURE 28G



FIGURE 28H



FIGURE 28I



FIGURE 28J



FIGURE 28K



FIGURE 28L

**ELECTRODE STRUCTURE AND METHOD  
FOR FORMING ELECTRODE STRUCTURE  
FOR A FLAT PANEL DISPLAY**

This is a division of application Ser. No. 09/421,781, filed Oct. 19, 1999.

**FIELD OF THE INVENTION**

The present claimed invention relates to the field of flat panel displays. More particularly, the present claimed invention relates to a method for forming an electrode structure for a flat panel display.

**BACKGROUND ART**

Display devices such as, for example, flat panel display devices typically utilize a cathode structure that is formed over a backplate. The cathode structure includes row electrodes and column electrodes that are used to activate regions of field emitters. The field emitters emit electrons that are directed towards respective pixel or sub-pixel regions on a faceplate. By selectively activating row electrodes and column electrodes, electrons are emitted that strike the respective pixel or sub-pixel regions on the faceplate. Typically, phosphors are coated on the inside of the faceplate. The electrons strike the phosphors, producing red, green or blue visible light that forms a visible display.

In prior art processing techniques, aluminum is commonly used for forming row electrodes and column electrodes. However, aluminum is subject to hillock formation. Hillock formation results in nonuniform planarization and can cause both row and column shorts to occur.

In one recent prior art process a layer of tantalum is deposited over the aluminum layer for reducing hillock formation. However, the resulting structure has a conductivity that is too low for use in large flat panel display devices. That is, though this process is sufficient for making small flat panel displays, the resulting row or column has too high a resistivity to be used in making large flat panel displays.

In prior art processes that use a layer of aluminum that is overlain by a layer of tantalum, the layer of aluminum is first deposited by placing the backplate into a sputtering chamber. Once the aluminum layer deposition is complete, the backplate is removed from the sputtering chamber. The layer of aluminum is then masked. More particularly, photoresist is deposited over the backplate, and the photoresist is exposed. The layer of aluminum is then etched using a wet etch process to form the desired aluminum structure.

The backplate is then placed into a second sputtering chamber that deposits the tantalum layer. Once the deposition of the tantalum layer is complete, the backplate is removed from the second sputtering chamber. The layer of tantalum is then masked. More particularly, photoresist is deposited over the backplate, and the photoresist is exposed. The tantalum layer is then etched. Because wet etch processes are not effective for etching tantalum, prior art processes must use a dry etch process. In one recent prior art process a reactive ion etch is used for etching the tantalum layer.

The use of two separate sputtering deposition steps is expensive and time consuming. Also, the use of two separate masking process steps is expensive and time consuming. These factors result in a low manufacturing yield and throughput. In addition, the steepness of the row electrodes and column electrodes of prior art processes results in

manufacturing defects related to cracking of the overlying tantalum layer.

The dry etch process is complex. Also, the use of a dry etch process is expensive as it requires the use of expensive capital equipment (e.g. reactive ion etcher). Moreover, the dry etch process is corrosive to aluminum and can result in corrosion of the aluminum layer when pinholes are present in the tantalum layer. In addition, the dry etch process forms polymers within the tantalum layer. Thus, following the dry etch, a polymer strip process is required for removing the polymers. The polymer strip process is expensive. In addition, the corrosive dry etch process can result in pinholes in the glass backplate.

During subsequent conventional process steps, the column electrode is subjected to potential damage. More particularly damage often results from, ion bombardment, cavity etch, cone deposition, dielectric deposition, masking and etching of the dielectric layer, deposition and etch of a molybdenum layer, deposition and etch of a chromium layer, polyimide deposition, etc. These process steps lead to shorts and opens that result in reduced yield and device failure.

Another problem that occurs in prior art devices is column to focus waffle shorts. These column to focus waffle shorts lead to reduced yield and device failure. In addition, the electrodes used in prior art column electrodes can react with the frit seal in the frit seal region, leading to shorts between column electrodes.

Thus, a need exists for an electrode structure and a method for forming an electrode structure that does not result in hillock formation. Still another need exists for an electrode structure and a method for forming an electrode structure that meets the above-listed needs but which does not produce undesired electrical shorts or opens in the cathode structure. Still another need exists for an electrode structure and a method for forming an electrode structure that meets the above-listed needs and that is inexpensive to manufacture and that does not result in reduced yield.

**SUMMARY OF INVENTION**

The present invention provides an electrode structure and a method for forming an electrode structure that does not result in hillock formation. Also, the present invention provides an electrode structure and a method for forming an electrode structure that meets the above-listed need but which does not produce undesired electrical shorts or opens in the cathode structure. Also, the present invention provides an electrode structure and a method for forming an electrode structure that meets the above-listed needs and that is inexpensive and that increases yield and throughput.

In one embodiment of the present invention, an electrode structure for a flat panel display is shown that includes lower electrodes and upper electrodes. In the present embodiment, the lower electrodes are row electrodes and the upper electrodes are column electrodes. The lower electrodes and the upper electrodes are separated by a resistive layer and a dielectric layer. In one embodiment, both the upper electrodes and the lower electrodes are formed of a metal alloy. In one embodiment, the metal alloy is an aluminum alloy. Alternatively, a silver alloy is used.

A method for forming an electrode structure of a flat panel display is disclosed. First, a metal alloy layer is deposited over a backplate. A cladding layer is then deposited over the metal alloy layer. A wet etch step is then performed so as to form a layer of electrodes. By performing the deposition of the metal alloy layer and the cladding layer in the same sputtering tool sequentially, cost savings, increased yield

and throughput result as compared to prior art processes that require two separate trips to a sputtering tool. Moreover, because a single masking step and a single wet etch is required, significant cost savings, increased yield and throughput result as compared to prior art processes that require two separate masking steps and etch steps.

The present invention does not use a dry etch process. Thus, significant cost savings are realized because there is no need for complex and expensive capital equipment for performing the dry etch process. In addition, because the present invention does not use a dry etch process, there is no corrosion of an underlying aluminum layer and no damage (e.g. pinholes) to the glass backplate. Moreover, because the present invention does not use a dry etch process, there is no need to perform a polymer strip process. This results in further time and cost savings as compared to prior art processes and increased throughput and yield.

In one embodiment, a passivation layer is deposited over the upper electrode. In the present embodiment, the passivation layer is silicon nitride. The silicon nitride layer is then masked and etched. The resulting silicon nitride structure partially covers the upper electrodes. This protects the upper electrodes during subsequent process steps.

Gate metal is then deposited, masked and etched to form a gate structure. The passivation layer protects the upper electrodes during deposition, mask and etch steps. Conventional process steps are then used to complete the cathode structure. In one embodiment of the present conventional process steps are used to form emitters and to form a focusing structure. In the present embodiment, these process steps include ion bombardment, cavity etch, cone deposition, dielectric deposition, masking and etching of the dielectric layer, deposition and etch of molybdenum layer, deposition and etch of chromium layer, polyimide deposition, etc. During these process steps, the upper electrodes are protected by the passivation layer. Thus, damage to upper electrodes is prevented. By preventing damage to upper electrodes, column shorts and opens are reduced. Also, because there is less exposed metal alloy, column to focus waffle shorts are decreased.

The use of either an aluminum alloy or the use of a silver alloy provides good conductivity. The resulting conductivity is sufficient for fabrication of large flat panel displays. In addition, the present invention prevents hillock formation as occurs in prior art processes that use aluminum. Thus, electrical shorts and opens are prevented as compared with prior art processes that use aluminum and good planarity of overlying layers is obtained. This results in increased yield as compared with prior art processes that use aluminum.

Thus, the present invention provides an electrode structure and a method for forming an electrode structure that does not result in hillock formation. Also, the present invention provides an electrode structure and a method for forming an electrode structure that meets the above-listed need but which does not produce undesired electrical shorts or opens in the cathode structure. Also, the present invention provides an electrode structure and a method for forming an electrode structure that meets the above-listed needs, that is inexpensive and that increases yield and throughput.

These and other objects and advantages of the present invention will no doubt become obvious to those of ordinary skill in the art after having read the following detailed description of the preferred embodiments which are illustrated in the various drawing figures.

#### BRIEF DESCRIPTION OF THE DRAWINGS

The accompanying drawings, which are incorporated in and form a part of this specification, illustrates embodiments

of the invention and, together with the description, serve to explain the principles of the invention:

FIG. 1 is a diagram showing a method for forming an electrode structure of a display device in accordance with one embodiment of the present invention.

FIG. 2 is a side sectional view of a display device showing a backplate over which a metal alloy layer is deposited in accordance with one embodiment of the present invention.

FIG. 3 is a side sectional view of a display device showing the deposition of a cladding layer in accordance with one embodiment of the present invention.

FIG. 4A is a side sectional view of a display device showing an expanded view of the structure of FIG. 3 after mask and etch steps have formed a lower electrode in accordance with one embodiment of the present claimed invention.

FIG. 4B is a side sectional view of a display device showing an expanded view of the structure of FIG. 3 after mask and etch steps have formed a lower electrode in accordance with one embodiment of the present claimed invention.

FIG. 5A is a side sectional view of a display device showing the structure of FIG. 4A after the deposition of a resistor layer in accordance with one embodiment of the present claimed invention.

FIG. 5B is a side sectional view of a display device showing the structure of FIG. 4B after the deposition of a resistor layer in accordance with one embodiment of the present claimed invention.

FIG. 6A is a side sectional view of a display device showing the structure of FIG. 5A after the deposition of a dielectric layer in accordance with one embodiment of the present claimed invention.

FIG. 6B is a side sectional view of a display device showing the structure of FIG. 5B after the deposition of a dielectric layer in accordance with one embodiment of the present claimed invention.

FIG. 7A is a side sectional view of a display device showing the structure of FIG. 6A after the deposition of a metal alloy layer in accordance with one embodiment of the present claimed invention.

FIG. 7B is a side sectional view of a display device showing the structure of FIG. 6B after the deposition of a metal alloy layer in accordance with one embodiment of the present claimed invention.

FIG. 8A is a side sectional view of a display device showing the structure of FIG. 7A after the deposition of a cladding layer in accordance with one embodiment of the present claimed invention.

FIG. 8B is a side sectional view of a display device showing the structure of FIG. 7B after the deposition of a cladding layer in accordance with one embodiment of the present claimed invention.

FIG. 9A is a side sectional view of a display device showing the structure of FIG. 8A after mask and etch steps have been performed in accordance with one embodiment of the present claimed invention.

FIG. 9B is a side sectional view of a display device showing the structure of FIG. 8B after mask and etch steps have been performed in accordance with one embodiment of the present claimed invention.

FIG. 10A is a side sectional view of a display device showing the structure of FIG. 9A after the deposition of a passivation layer in accordance with one embodiment of the present claimed invention.

FIG. 10B is a side sectional view of a display device showing the structure of FIG. 9B after the deposition of a passivation layer in accordance with one embodiment of the present claimed invention.

FIG. 11A is a side sectional view of a display device showing the structure of FIG. 10A after mask and etch steps have been performed in accordance with one embodiment of the present claimed invention.

FIG. 11B is a side sectional view of a display device showing the structure of FIG. 10B after mask and etch steps have been performed in accordance with one embodiment of the present claimed invention.

FIG. 12A is a side sectional view of a display device showing the structure of FIG. 11A after deposition of a gate metal layer in accordance with one embodiment of the present claimed invention.

FIG. 12B is a side sectional view of a display device showing the structure of FIG. 11B after deposition of a gate metal layer in accordance with one embodiment of the present claimed invention.

FIG. 13A is a side sectional view of a display device showing the structure of FIG. 12A after mask and etch steps have been performed in accordance with one embodiment of the present claimed invention.

FIG. 13B is a side sectional view of a display device showing the structure of FIG. 12B after mask and etch steps have been performed in accordance with one embodiment of the present claimed invention.

FIG. 14A is a side sectional view of a display device showing the structure of FIG. 13A after formation of emitters and focus structure in accordance with one embodiment of the present claimed invention.

FIG. 14B is a side sectional view of a display device showing the structure of FIG. 13B after formation of emitters and focus structure in accordance with one embodiment of the present claimed invention.

FIG. 15 is a diagram showing a method for forming an electrode structure of a display device in accordance with one embodiment of the present invention.

FIG. 16A is a side sectional view of a display device showing a backplate over which lower and upper electrodes are formed and having a resistor layer, a dielectric layer, and a gate structure in accordance with one embodiment of the present claimed invention.

FIG. 16B is a side sectional view of a display device showing a backplate over which lower and upper electrodes are formed and having a resistor layer, a dielectric layer, and a gate structure in accordance with one embodiment of the present claimed invention.

FIG. 16C is a side sectional view of a display device showing the structure of FIG. 9A after deposition, mask and etch have formed a passivation layer in accordance with one embodiment of the present claimed invention.

FIG. 16D is a side sectional view of a display device showing the structure of FIG. 9B after deposition, mask and etch have formed a passivation layer in accordance with one embodiment of the present claimed invention.

FIG. 16E is a side sectional view of a display device showing the structure of FIG. 16C after mask and etch steps have been performed in accordance with one embodiment of the present claimed invention.

FIG. 16F is a side sectional view of a display device showing the structure of FIG. 16D after mask and etch steps have been performed in accordance with one embodiment of the present claimed invention.

FIG. 16G is a side sectional view of a display device showing the structure of FIG. 16E after evaporation of a chromium layer and deposition of cone material, deposition of a layer of dielectric material, and mask and etch steps have been performed in accordance with one embodiment of the present claimed invention.

FIG. 16H is a side sectional view of a display device showing the structure of FIG. 16F after evaporation of a chromium layer and deposition of cone material, deposition of a layer of dielectric material, and mask and etch steps have been performed in accordance with one embodiment of the present claimed invention.

FIG. 16I is a side sectional view of a display device showing a completed cathode structure in accordance with one embodiment of the present claimed invention.

FIG. 16J is a side sectional view of a display device showing a completed cathode structure in accordance with one embodiment of the present claimed invention.

FIG. 17 is a diagram showing a method for forming an electrode structure of a display device in accordance with one embodiment of the present invention.

FIG. 18A is a side sectional view of a display device showing a backplate over which lower and upper electrodes are formed and having a resistor layer, a dielectric layer, and a gate layer in accordance with one embodiment of the present claimed invention.

FIG. 18B is a side sectional view of a display device showing a backplate over which lower and upper electrodes are formed and having a resistor layer, a dielectric layer, and a gate layer in accordance with one embodiment of the present claimed invention.

FIG. 18C is a side sectional view of a display device showing the structure of FIG. 18A after mask and etch steps have formed a gate structure in accordance with one embodiment of the present claimed invention.

FIG. 18D is a side sectional view of a display device showing the structure of FIG. 18B after mask and etch steps have formed a gate structure in accordance with one embodiment of the present claimed invention.

FIG. 18E is a side sectional view of a display device showing the structure of FIG. 18C after mask and etch steps have been performed in accordance with one embodiment of the present claimed invention.

FIG. 18F is a side sectional view of a display device showing the structure of FIG. 18D after mask and etch steps have been performed in accordance with one embodiment of the present claimed invention.

FIG. 18G is a side sectional view of a display device showing the structure of FIG. 18E after the deposition of a passivation layer and after mask and etch steps have been performed in accordance with one embodiment of the present claimed invention.

FIG. 18H is a side sectional view of a display device showing the structure of FIG. 18F after the deposition of a passivation layer and after mask and etch steps have been performed in accordance with one embodiment of the present claimed invention.

FIG. 18I is a side sectional view of a display device showing the structure of FIG. 18G after evaporation of a chromium layer and deposition of cone material, deposition of a layer of dielectric material, and mask and etch steps have been performed in accordance with one embodiment of the present claimed invention.

FIG. 18J is a side sectional view of a display device showing the structure of FIG. 18H after evaporation of a





## 11

FIG. 26K is a side sectional view of a display device showing the structure of FIG. 26I after mask and etch steps have been performed in accordance with one embodiment of the present claimed invention.

FIG. 26L is a side sectional view of a display device showing the structure of FIG. 26J after mask and etch steps have been performed in accordance with one embodiment of the present claimed invention.

FIG. 27 is a diagram showing a method for forming an electrode structure of a display device in accordance with one embodiment of the present invention.

FIG. 28A is a side sectional view of a display device showing a backplate over which lower and upper electrodes are formed and having a resistor layer, a dielectric layer, a gate structure, an evaporated chromium layer, an evaporated molybdenum layer, and a dielectric layer in accordance with one embodiment of the present claimed invention.

FIG. 28B is a side sectional view of a display device showing a backplate over which lower and upper electrodes are formed and having a resistor layer, a dielectric layer, a gate structure, an evaporated chromium layer, an evaporated molybdenum layer, and a dielectric layer in accordance with one embodiment of the present claimed invention.

FIG. 28C is a side sectional view of a display device showing the structure of FIG. 28A after mask and etch steps have been performed in accordance with one embodiment of the present claimed invention.

FIG. 28D is a side sectional view of a display device showing the structure of FIG. 28B after mask and etch steps have been performed in accordance with one embodiment of the present claimed invention.

FIG. 28E is a side sectional view of a display device showing the structure of FIG. 28C after mask and etch steps have been performed in accordance with one embodiment of the present claimed invention.

FIG. 28F is a side sectional view of a display device showing the structure of FIG. 28D after mask and etch steps have been performed in accordance with one embodiment of the present claimed invention.

FIG. 28G is a side sectional view of a display device showing the structure of FIG. 28E after focusing structures have been formed in accordance with one embodiment of the present claimed invention.

FIG. 28H is a side sectional view of a display device showing the structure of FIG. 28F focusing structures have been formed in accordance with one embodiment of the present claimed invention.

FIG. 28I is a side sectional view of a display device showing the structure of FIG. 28G after an etch step has been performed in accordance with one embodiment of the present claimed invention.

FIG. 28J is a side sectional view of a display device showing the structure of FIG. 28H after an etch step has been performed in accordance with one embodiment of the present claimed invention.

FIG. 28K is a side sectional view of a display device showing the structure of FIG. 28I after an etch step has been performed in accordance with one embodiment of the present claimed invention.

FIG. 28L is a side sectional view of a display device showing the structure of FIG. 26J after an etch step has been performed in accordance with one embodiment of the present claimed invention.

The drawings referred to in this description should be understood as not being drawn to scale except if specifically noted.

## 12

## DESCRIPTION OF THE PREFERRED EMBODIMENTS

Reference will now be made in detail to the preferred embodiments of the invention, examples of which are illustrated in the accompanying drawings. While the invention will be described in conjunction with the preferred embodiments, it will be understood that they are not intended to limit the invention to these embodiments. On the contrary, the invention is intended to cover alternatives, modifications and equivalents, which may be included within the spirit and scope of the invention as defined by the appended claims. Furthermore, in the following detailed description of the present invention, numerous specific details are set forth in order to provide a thorough understanding of the present invention. However, it will be obvious to one of ordinary skill in the art that the present invention may be practiced without these specific details. In other instances, well known methods, procedures, components, and circuits have not been described in detail as not to unnecessarily obscure aspects of the present invention.

With reference now to FIG. 1, a method for forming an electrode structure for a display device is shown. As shown by step 101, a metal alloy layer is deposited. FIG. 2 shows a metal alloy layer 2 deposited over glass plate 1.

In one embodiment, metal alloy layer 2 is an aluminum alloy. In one embodiment, metal alloy layer 2 has a thickness of 500–5000 Angstroms. In one specific embodiment, an aluminum alloy is used that includes aluminum (Al) and Neodymium (Nd). In the present embodiment, the aluminum alloy has a concentration of from 0.5 to 6 atomic percent Nd. In another embodiment, an aluminum alloy is used that has a concentration of from 0.5 to 6 atomic percent Nd and from 0 to 5 atomic percent titanium (Ti).

Continuing with FIGS. 1–2, in an alternate embodiment, metal alloy layer 2 is a silver alloy. In one embodiment a silver alloy is used that includes silver (Ag) and 0.5 to 2 atomic percent palladium (Pd) and 0.5 to 2 atomic percent copper (Cu). In yet another embodiment, a silver alloy is used that includes 0.5 percent to 2 atomic percent palladium and 0.0 to 2.0 atomic percent titanium.

When a silver alloy is used, an adhesion layer can be used to promote adhesion to the glass plate. In one embodiment, a molybdenum adhesion layer is used that has a thickness of approximately 500–1000 angstroms.

Referring to FIG. 1, as shown by step 102, a cladding layer is then deposited. FIG. 3 shows the structure of FIG. 2 after cladding layer 3 has been deposited. It can be seen that cladding layer 3 directly overlies metal alloy layer 2.

In one embodiment, cladding layer 3 of FIG. 3 is a molybdenum (Mo) tungsten (W) alloy. In the present embodiment, cladding layer 3 has a thickness of approximately 500–4000 angstroms. The use of cladding layer 3 produces a contact pad that is reliable and that maintains good electrical contact. In addition, the use of cladding layer 3 further reduces hillock formation.

Though the present invention includes the deposition of cladding layer 3, the present invention is well adapted for use without cladding layer 3. That is, the use of aluminum alloy or silver alloy provides sufficient reduction in hillock formation and results in good conductivity as compared with prior art processes.

In one embodiment, a diffusion barrier layer is used. The diffusion barrier layer can be formed of is titanium, titanium nitride or titanium tungsten that is deposited directly over

13

the silver alloy. In one embodiment, a diffusion barrier layer is used that has a thickness of approximately 500–2000 Angstroms. The use of a diffusion barrier layer is particularly useful in an embodiment that does not include a cladding layer.

In one embodiment, the deposition of metal alloy layer 2 and cladding layer 3 is conducted using a single sputtering tool. That is, in the present invention, a sputtering process is used whereby metal alloy layer 2 and cladding layer 3 are sequentially deposited in a single sputtering tool. More particularly, in one embodiment, glass plate 1 is placed into a sputtering tool that includes a sputtering chamber that first deposits metal alloy layer 2 and then deposits cladding layer 3. The glass plate is then removed from the sputtering chamber. This provides significant cost savings over prior art methods that require two separate sputtering process steps and results in increased throughput and yield.

The use of either an aluminum alloy or the use of a silver alloy in conjunction with a cladding layer provides good conductivity. The resulting conductivity is sufficient for fabrication of large flat panel displays. In addition, the present invention prevents hillock formation as occurs in prior art processes that use aluminum. Thus, shorts are prevented as compared with prior art processes that use aluminum and planarity of overlying layers is obtained. This results in increased yield as compared with prior art processes that use aluminum.

Referring back to FIG. 1, mask and etch steps are performed as shown by step 103. More particularly, in the present embodiment, photoresist is deposited over the backplate and is patterned. The backplate is then etched using a wet etch process to form the desired row electrodes. FIGS. 4A–4B show the structure of FIG. 3 after mask and etch steps have formed exemplary lower electrode 4.

The present invention requires a single patterning step and a single etch step in order to form row electrodes. Thus, the present invention does not require two separate patterning steps as are required in prior art processes. This results in significant cost savings as compared to prior art processes that require two separate patterning steps. In addition, because the present invention does not require two separate etch steps as are required in prior art processes that use a molybdenum cap, the present invention results in increased yield and throughput.

The present invention does not use a dry etch process for forming row electrodes. Thus, significant cost savings are realized because there is no need for complex and expensive capital equipment for performing the dry etch process. In addition, because the present invention does not use a dry etch process, there is no corrosion of an underlying aluminum layer and no damage (e.g. pinholes) to the glass backplate. Moreover, because the present invention does not use a dry etch process, there is no need to perform a polymer strip process. This results in further increases in throughput and yield as compared to prior art processes.

In one embodiment, the etching process forms angled edges. In the present embodiment, an etchant is used that includes nitric acid, phosphoric acid, ascetic acid and water. The use of this etchant performs a controlled lifting of the photoresist and results in angled edges on the sides of the lower electrode 4. The use of angled edges results in good conformity of overlying layers and reduces cracking in overlying layers.

Referring back to FIG. 1, a resistor layer is deposited as shown by step 104. In the embodiment shown in FIGS. 5A–5B, resistor layer 5 is shown to overlie lower electrode

14

4. In one embodiment, resistor layer 5 has a thickness of approximately 2000 angstroms. In the present embodiment, resistor layer 5 is silicon carbide (SiC) that is either deposited using a sputtering process or a chemical vapor deposition process.

A layer of dielectric is then deposited as shown by step 105 of FIG. 1. In one embodiment silicon dioxide (SiO<sub>2</sub>) is used as a dielectric. In the present embodiment, a plasma enhanced chemical vapor deposition process is used to 10 deposit the silicon dioxide layer. Referring now to FIGS. 6A–6B, the embodiment of FIGS. 5A–5B is shown after the deposit of dielectric layer 6.

A metal alloy layer is then deposited as shown by step 106 of FIG. 1. In the present embodiment, the metal alloy layer 15 has a thickness of approximately 500–5000 Angstroms. FIGS. 7A–7B show metal alloy layer 11 deposited over dielectric layer 6. In one embodiment, metal alloy layer 11 is an aluminum alloy. More particularly, in one specific embodiment, an aluminum alloy is used that includes aluminum and from 0.5 to 6 atomic percent neodymium and from 0 to 5 atomic percent titanium.

Alternatively, metal alloy layer 11 is a silver alloy. In one embodiment, metal alloy layer 11 includes silver and 0.5 to 2 atomic percent palladium and 0.5 to 2 atomic percent copper. In yet another embodiment, a silver alloy is used that includes 0.5 percent to 2 atomic percent palladium Pd and 0.0 to 2.0 atomic percent titanium.

When a silver alloy is used an adhesion layer can be used to promote adhesion to the gate structure. In one embodiment, a molybdenum adhesion layer is used that has a thickness of approximately 500–1000 angstroms is used.

Referring to FIG. 1, as shown by step 107, a cladding layer is then deposited. FIGS. 8A–8B shows the structure of FIGS. 7A–7B after cladding layer 12 has been deposited. It can be seen that cladding layer 12 directly overlies metal alloy layer 11.

In one embodiment, cladding layer 12 of FIG. 3 is a molybdenum tungsten alloy. In the present embodiment, cladding layer 12 has a thickness of approximately 40 500–4000 angstroms. The use of cladding layer 12 produces a contact pad that is reliable and that maintains good electrical contact. In addition, the use of cladding layer 12 further reduces hillock formation.

Though the present invention includes the deposition of cladding layer 12, the present invention is well adapted for use without cladding layer 12. That is, the use of aluminum alloy or silver alloy provides sufficient reduction in hillock formation and results in good conductivity as compared with prior art processes. In an embodiment that does not include cladding layer 12 but which uses a silver alloy, a diffusion barrier layer can be used. In one embodiment, the diffusion barrier layer is titanium or titanium nitride or titanium tungsten that is deposited over the silver alloy and that has a thickness of approximately 500–2000 Angstroms.

In one embodiment, the deposition of metal alloy layer 11 and cladding layer 12 is conducted using a single sputtering tool. This provides significant cost savings over prior art methods that require two separate sputtering process steps and results in increased throughput and yield.

Referring to step 108 of FIG. 1, mask and etch steps are performed for forming upper electrodes. In the present invention, a wet etch process is used. FIGS. 9A–9B show the structure of FIGS. 8A–8B after mask and etch steps have 65 formed exemplary upper electrode 14. In one embodiment, an etchant is used that includes nitric acid, phosphoric acid, ascetic acid and water for forming angled edges on the sides

## 15

of upper electrode 14. The use of an angled edges results in good conformity of overlying layers and reduces cracking in overlying layers.

The use of either an aluminum alloy or the use of a silver alloy in conjunction with a cladding layer provides good conductivity. The resulting conductivity is sufficient for fabrication of large flat panel displays. In addition, the present invention prevents hillock formation as occurs in prior art processes that use aluminum. Thus, shorts are prevented as compared with prior art processes that use aluminum and planarity of overlying layers is obtained. This results in increased yield as compared with prior art processes that use aluminum. Moreover, the present invention requires a single patterning step and a single etch step in order to form upper electrode 14. Thus, the present invention does not require two separate patterning steps and two separate etch steps as are required in prior art processes. This results in significant cost savings and increased yield and throughput. Also, the present invention does not use a dry etch process. This results in cost savings and increases in yield and throughput.

Referring now to step 109 of FIG. 1, a passivation layer is deposited. In one embodiment, the passivation layer is silicon nitride deposited using a plasma enhanced chemical vapor deposition process. Referring now to

FIGS. 10A–10B, the structure of FIGS. 9A–9B is shown after passivation layer 15 is deposited.

Referring now to step 110 of FIG. 1, mask and etch steps are performed. FIGS. 11A–11B show the structure of FIGS. 10A–10B after mask and etch steps have formed openings 16–18. It can be seen that passivation layer 15 extends over upper electrode 14 except at openings 17–18.

Gate metal is then deposited as shown by step 111 of FIG. 1. In one embodiment, chromium is used as a gate metal. FIGS. 12A–12B show the structure of FIGS. 11A–11B after gate metal layer 20 has been deposited. In an alternate embodiment, gate metal layer 20 is formed by first depositing a tantalum layer and then depositing a chromium layer over the tantalum layer. Passivation layer 15 protects upper electrode 14 during the deposition of gate metal layer 20.

Referring now to step 112 of FIG. 1, mask and etch steps are performed to form a gate structure. FIGS. 13A–13B show the structure of FIGS. 11A–11B after mask and etch steps have formed gate structure 21. In the present embodiment, column contact pad 22 allows for contact with upper electrode 14. Passivation layer 15 protects upper electrode 14 during mask and etch steps for forming gate metal structure 21.

Conventional process steps are then used to complete the cathode structure as shown by step 113 of FIG. 1. FIGS. 14A–14B show a completed cathode structure according to one embodiment of the present invention. In one embodiment of the present conventional process steps are used to form cavity 221 and to form exemplary emitter 26 within cavity 221. Mask and etch steps are used to extend opening 16 of FIG. 11B so as to expose row contact pad 23. Conventional process steps are also used to form focusing structure 24 and focus waffle metal 27. In one embodiment, focus waffle metal 27 is aluminum. In the present invention, these process steps include ion bombardment, cavity etch, cone deposition, dielectric deposition, masking and etching of the dielectric layer, polyimide deposition, etc.

During the process steps for completion of the cathode, upper electrode 14 is protected by passivation layer 15. This prevents damage to upper electrode 14 as typically occurs in prior art processes. By preventing damage to upper electrode

## 16

14, upper electrode shorts and opens are prevented. In addition, because upper electrode 14 is protected, column shorts in the frit seal region are eliminated. Also, because there is less exposed metal as compared with prior art processes, column to focus waffle shorts are decreased.

With reference now to FIGS. 15a–f, a second embodiment of a method for forming an electrode structure for a display device is shown. As shown by step 101 a metal alloy layer is deposited. As shown by step 102, a cladding layer is then deposited. Mask and etch steps are performed as shown by step 103 to form lower electrodes. A resistor layer is deposited as shown by step 104. A layer of dielectric is then deposited as shown by step 105. A metal alloy layer is then deposited as shown by step 106. As shown by step 107, a cladding layer is then deposited. Referring to step 108, mask and etch steps are performed for forming upper electrodes. In one embodiment, steps 101–108 are identical to steps 101–108 of FIG. 1, producing the structure shown in FIGS. 9A–9B.

Referring now to step 111 of FIG. 15, a gate metal layer is deposited. The gate metal layer is then masked and etched as shown by step 112. Referring now to FIGS. 16a–b, the structure of FIGS. 9a–9b is shown after steps 111–112 have been performed so as to form gate structure 1601. In one embodiment, gate structure 1601 is chromium. Alternatively, gate structure 1601 is a layer of chromium deposited over a layer of tantalum.

Continuing with FIG. 15, as shown by steps 109–110, a passivation layer is deposited, masked and etched. FIGS. 16c–16d show the structure of FIGS. 16a–16b after steps 109–110 have formed passivation layer 1602. In one embodiment, passivation layer 1602 is silicon nitride deposited using a plasma enhanced chemical vapor deposition process. Openings 1620–1621 extend through passivation layer 1602. It can be seen that passivation layer 1602 extends over gate structure 1601 except at openings 1620–1621.

The cathode structure is then completed as shown by step 113 of FIG. 15. FIGS. 16E–16J illustrate an exemplary method for completing the cathode structure in accordance with one embodiment of the present invention. First an etch step is performed. FIGS. 16E–16F show the structure of FIGS. 16C–16D after the etch step has formed cavity 25. A layer of chromium is evaporated over the structure, followed by the deposition of cone material and the deposition of a dielectric layer. In one embodiment, the layer of chromium is thin, having a thickness of approximately 500 Angstroms. The resulting structure is then patterned and etched so as to produce the structure shown in FIGS. 16G–16H. The structure of FIGS. 16G–16H shows dielectric material 1654, cone 26, cone material 1653 and chromium 1640. In one embodiment, cone material 1653 is evaporated molybdenum. However, the present invention is well adapted for use of other materials for forming cone 26. Mask and etch steps form opening 1656 that exposes portions of lower electrode 4 so as to form lower contact pad 23. Dielectric removal steps and a halo etch are then performed, followed by formation of polyimide structures and focus waffle metal. FIGS. 16I–16J show a completed cathode structure that includes polyimide structures 24, focus waffle metal 27 and upper contact pad 22.

During the process steps for completion of the cathode, upper electrode 14 is protected by gate metal structure 1601 and by passivation layer 15. This prevents damage to upper electrode 14 as typically occurs in prior art processes. By preventing damage to upper electrode 14, upper electrode

shorts and opens are prevented. In addition, because upper electrode 14 is protected, column shorts in the frit seal region are eliminated. Also, because there is less exposed metal as compared with prior art processes, column to focus waffle shorts are decreased.

With reference now to FIG. 17, yet another method for forming an electrode structure for a display device is shown. As shown by step 201, lower electrodes are formed over a substrate. A resistor layer and a dielectric layer are then deposited over the lower electrodes as shown by steps 202–203. In one embodiment, steps 201–203 are identical to steps 101–105 of FIG. 1.

Continuing with FIG. 17, gate metal is deposited as is shown by step 204. In one embodiment, chromium is used as a gate metal.

Referring still to FIG. 17, upper electrodes are formed as shown by step 205. In the one embodiment, upper electrodes are formed in the same manner as shown in steps 106–108 of FIGS. 1 and 15. In the present embodiment, upper electrodes are formed by depositing a metal alloy layer that is an aluminum alloy and masking and etching the metal alloy layer. In one specific embodiment, a metal alloy layer is used that a thickness of 500–5000 Angstroms and that includes aluminum (Al) and Neodymium (Nd) with a concentration of from 0.5 to 6 atomic percent Nd. In another embodiment, an aluminum alloy is used that has a concentration of from 0.5 to 6 atomic percent Nd and from 0 to 5 atomic percent titanium (Ti).

FIGS. 18A–18B show substrate 1 after steps 201–205 have been performed, forming lower electrodes 4 over substrate 1, resistor layer 5, dielectric layer 6, gate metal layer 1801 and upper electrodes 1810.

Referring back to FIG. 17, as shown by step 206, mask and etch steps are then performed so as to selectively etch gate metal layer 1801 of FIGS. 18A–18B. More particularly, in the present embodiment, photoresist is deposited over the backplate and is patterned. The backplate is then etched using a wet etch process. FIGS. 18C–18D show the structure of FIGS. 18A–18B after mask and etch steps have formed gate metal structure 1811.

Referring now to step 207 of FIG. 17, a passivation layer is deposited. In one embodiment, the passivation layer is silicon nitride deposited using a plasma enhanced chemical vapor deposition process.

Referring now to step 208 of FIG. 17, mask and etch steps are performed. Referring now to FIGS. 18E–18F, the structure of FIGS. 18C–18D is shown after a passivation layer is deposited, masked and etched to form openings 1820 and 1821 that extend through passivation layer 1830. In one embodiment of the present invention, cavity 1825 is also formed using a HALO etch. It can be seen that passivation layer 1830 extends over upper electrode 1810 except at opening 1820.

The cathode structure is then completed as shown by step 209 of FIG. 17. FIGS. 18G–18N illustrate an exemplary method for completing the cathode in accordance with one embodiment of the present invention. Mask and etch steps are performed to form a cavity, shown in FIG. 18G as cavity 1825. A layer of chromium is evaporated over the structure, followed by the deposition of cone material and the deposition of a dielectric layer. The resulting structure is then patterned and etched so as to produce the structure shown in FIGS. 18I–18J. More particularly, cone 1826 and structures 1891 and 1892 are formed. Structures 1891 and 1892 include cone material 1853, chromium material 1840 and dielectric material 1854. Mask and etch steps then form

openings that expose portions of lower electrode 4 so as to form lower contact pad 1856 as shown in FIGS. 18K–18L. Dielectric removal steps and a halo etch are then performed, followed by formation of polyimide structures and focus waffle metal. FIGS. 18M–18N show a completed cathode structure that includes upper contact pad 1857, focusing structures 1824 and focus waffle metal 1827. In an alternate embodiment of the present invention (not shown) mask and etch steps do not form structure 1892. That is, only structure 1891 is formed.

During the process steps for completion of the cathode, upper electrode 1810 is protected by passivation layer 1830. This prevents damage to upper electrode 1810 as typically occurs in prior art processes. By preventing damage to upper electrode 1810, upper electrode shorts and opens are prevented. In addition, because upper electrode 1810 is protected, column shorts in the frit seal region are eliminated. Also, because there is less exposed metal as compared with prior art processes, column to focus waffle shorts are decreased.

With reference now to FIG. 19, yet another method for forming an electrode structure for a display device is shown. As shown by step 201 lower electrodes are formed over a substrate. A resistor layer and a dielectric layer are then deposited over the lower electrodes as shown by steps 202–203.

Continuing with FIG. 19, gate metal is deposited as is shown by step 204. In one embodiment, chromium is used as a gate metal.

Referring still to FIG. 19, a tantalum layer is deposited as shown by step 250. Upper electrodes are then formed as shown by step 205. In the present embodiment, upper electrodes are formed using an aluminum alloy. In one embodiment, the metal alloy has a thickness of 500–5000 Angstroms. In one specific embodiment, an aluminum alloy is used that includes aluminum (Al) and Neodymium (Nd). In the present embodiment, the aluminum alloy has an concentration of from 0.5 to 6 atomic percent Nd. In another embodiment, an aluminum alloy is used that has a concentration of from 0.5 to 6 atomic percent Nd and from 0 to 5 atomic percent titanium (Ti).

FIGS. 18a–18b show substrate 1 after steps 201–205 and 250 have been performed, forming a gate metal layer 1801, a tantalum layer 1802, and upper electrodes 1810. In one embodiment, lower electrode 4 is a row electrode and upper electrode 1810 is a column electrode. However, alternatively, the present invention is well adapted to use of lower electrode 4 as a column electrode and upper electrode 1810 as a row electrode.

Referring back to FIG. 19, as shown by step 252, mask and etch steps are then performed so as to selectively etch tantalum layer 1802 and gate metal layer 1801 of FIGS. 20A–20B. More particularly, in the present embodiment, photoresist is deposited over the backplate and is patterned. The backplate is then etched using a wet etch process. FIGS. 20C–20D show the structure of FIGS. 20A–20B after mask and etch steps have formed gate metal structure 1811 and tantalum structure 1812.

Referring now to step 207 of FIG. 19, a passivation layer is deposited. In one embodiment, the passivation layer is silicon nitride deposited using a plasma enhanced chemical vapor deposition process.

Referring now to step 208 of FIG. 19, mask and etch steps are performed. Referring now to FIGS. 20E–20F, the structure of FIGS. 20C–20D is shown after a passivation layer is deposited, masked and etched to formed opening 1820 that

## 19

extends through passivation layer 1830 and tantalum structure 1812. In one embodiment of the present invention, a halo etch is also performed, forming cavity 1825. It can be seen that passivation layer 1830 extends over upper electrode 1810 except at opening 1820. Passivation layer 1830 protects upper electrode 1810 during subsequent process steps.

The cathode structure is then completed as shown by step 209 of FIG. 19. FIGS. 20G-20L illustrate an exemplary method for completing the cathode structure in accordance with one embodiment of the present invention. A layer of chromium is evaporated over the structure, followed by the deposition of cone material and the deposition of a dielectric layer. The resulting structure is then patterned and etched so as to produce the structure shown in FIGS. 20G-20H. The structure of FIGS. 20G-20H includes dielectric material 1854, cone 1826, cone material 1853 and chromium segment 1840. In one embodiment, cone material 1853 is evaporated molybdenum. However, the present invention is well adapted for use of other materials for forming cone 1826. Mask and etch steps then form openings 1856-1857 that expose portions of lower electrode 4 and upper electrode 1810 so as to form lower contact pad 1823 and upper contact pad 1822 as shown in FIGS. 20I-20J. Dielectric removal steps and a halo etch are then performed, followed by formation of polyimide structures and focus waffle metal. FIGS. 20K-20L show a completed cathode structure that includes polyimide structures 1824 and focus waffle metal 1827.

During the process steps for completion of the cathode, upper electrode 1810 is protected by passivation layer 1830. This prevents damage to upper electrode 1810 as typically occurs in prior art processes. By preventing damage to upper electrode 1810, upper electrode shorts and opens are prevented. In addition, because upper electrode 1810 is protected, column shorts in the frit seal region are eliminated. Also, because there is less exposed metal as compared with prior art processes, column to focus waffle shorts are decreased.

With reference now to FIG. 21, yet another method for forming an electrode structure for a display device is shown. As shown by steps 201, lower electrodes are formed over a substrate. A resistor layer and a dielectric layer are then deposited over the lower electrodes as shown by steps 202-203.

Continuing with FIG. 21, gate metal is deposited as is shown by step 204. In one embodiment, chromium is used as a gate metal. Upper electrodes are then formed as shown by step 205. In the present embodiment, upper electrodes are formed of an aluminum alloy. In one embodiment, steps 201-205 are identical to steps 201-205 of FIG. 17.

Referring now to FIGS. 22A-22B, a substrate 1 is shown after steps 201-205 have formed a gate metal layer 1801 and upper electrodes 1810 that overlie dielectric layer 6, resistor layer 5 and lower electrode 4.

Referring now to step 207 of FIG. 21, a passivation layer is deposited. In one embodiment, the passivation layer is silicon nitride deposited using a plasma enhanced chemical vapor deposition process. Alternatively, a tantalum layer can be used.

Referring back to FIG. 21, as shown by step 260, mask and etch steps are then performed. In one embodiment, a two step etch process is used whereby the passivation layer is etched using a first etch step and the gate metal layer is etched in a second etch step. The first mask and etch step etches through the passivation layer and etches through the

## 20

gate metal layer. FIGS. 22C-22D show the structure of FIGS. 22A-22B after mask and etch steps have formed gate metal structure 1811 and passivation layer 1830.

The cathode structure is then completed as shown by step 209 of FIG. 21. FIGS. 22E-22N illustrate an exemplary method for completing the cathode in accordance with one embodiment of the present invention. A dielectric layer is deposited over the structure of FIGS. 22C-22D. The dielectric layer 2250 is then patterned and etched to form the structure shown in FIGS. 22E-22F. During the etch process, passivation layer 1830 acts as an etch stop. A cavity etch is then performed. FIGS. 22G-22H show the structure of FIGS. 22E-22F after the cavity etch has formed cavity 1825.

A layer of Molybdenum is then deposited, using a sputter deposition process. A layer of cone material is then deposited over the layer of Molybdenum. In one embodiment, a cone material that is evaporated molybdenum is used. However, the present invention is well adapted for use of other materials for forming a cone. A layer of dielectric is then deposited. The resulting structure is then patterned and etched so as to produce the structure shown in FIGS. 22I-22J. The structure of FIGS. 22I-22J includes Molybdenum structure 2252, cone 2226, cone material 2253 and dielectric layer 2254. Mask and etch steps then form openings 2256-2257 shown in FIGS. 22K-22L. Referring now to FIGS. 22M-22N, dielectric removal steps and a halo etch are then performed, producing contact pads 2222 and 2223, followed by formation of polyimide focusing structures 2224 and focus waffle metal 2227.

During the process steps for completion of the cathode, upper electrode 1810 is protected by passivation layer 1830. This prevents damage to upper electrode 1810 as typically occurs in prior art processes. By preventing damage to upper electrode 1810, upper electrode shorts and opens are prevented. In addition, because upper electrode 1810 is protected, column shorts in the frit seal region are eliminated. Also, because there is less exposed metal as compared with prior art processes, upper electrode to focus waffle shorts are decreased.

With reference now to FIGS. 23-24, yet another method for forming an electrode structure for a display device is shown. As shown by step 201 of FIG. 23, lower electrodes are formed over a substrate. A resistor layer and a dielectric layer are then deposited over the lower electrodes as shown by steps 202-203. A gate metal layer is deposited as shown by step 204, followed by the formation of upper electrodes as shown by step 205. An etch step is then performed to form a gate structure as shown by step 206 followed by etch step 2301 to form a cavity.

In the present embodiment, upper electrodes are formed by the deposition and etch of a metal alloy layer. In one embodiment, the metal alloy is an aluminum alloy that has a thickness of 500-5000 Angstroms. In one specific embodiment, an aluminum alloy is used that includes aluminum (Al) and Neodymium (Nd). In the present embodiment, the aluminum alloy has a concentration of from 0.5 to 6 atomic percent Nd. In another embodiment, an aluminum alloy is used that has a concentration of from 0.5 to 6 atomic percent Nd and from 0 to 5 atomic percent titanium (Ti).

Referring to FIGS. 24A-24B, a substrate 1 is shown after steps 201-206 have formed lower electrodes 4, resistor layer 5, dielectric layer 6, gate metal structure 1811 and upper electrodes 1810. Etch step 2301 forms cavity 2425.

Continuing with FIG. 23, a layer of sputtered molybdenum is then deposited as shown by step 2302. A layer of

## 21

evaporated molybdenum is then deposited as shown by step 2303, followed by the deposition of a layer of sputtered molybdenum as shown by step 2304. Referring now to FIGS. 24C–24D, the structure of FIGS. 24A–24B is shown after steps 2302–2304 form sputtered molybdenum layer 2401, evaporated molybdenum layer 2402, sputtered molybdenum layer 2403 and cone 2426.

Referring back to FIG. 23, as shown by step 2305, mask and etch steps are then performed. FIGS. 24E–24F show the structure of FIGS. 24C–24D after mask and etch steps have formed molybdenum structures 2430–2431 and an opening 2422 that extends to the top of lower electrode 4. In one embodiment, mask and etch step 2305 includes two separate mask and etch steps, a first mask and etch step that etches sputtered molybdenum layer 2403, evaporated molybdenum 2402 and molybdenum layer 2401, and a second mask and etch step that etches through dielectric layer 6 and resistor layer 5 to form opening 2422.

Referring to step 2306 of FIG. 23, a dielectric layer is deposited. In one embodiment, the dielectric layer is silicon dioxide.

Referring now to step 2307 of FIG. 23, a passivation layer is deposited. In one embodiment, the passivation layer is silicon nitride deposited using a plasma enhanced chemical vapor deposition process. FIGS. 24G–24H show the structure of FIGS. 24E–24F after the deposition of dielectric layer 2440 and passivation layer 2441.

Referring now to step 2308, mask and etch steps are then performed. Referring now to FIGS. 24I–24J step 2308 forms openings 2450–2452 that extend through passivation layer 2441.

As shown in step 2309, focusing structures are formed. A dry etch process is then performed as shown by step 2310. Referring now to FIGS. 24K–24L, steps 2309–2310 form polyimide focusing structures 2424 and openings 2461–2463 that extend through dielectric layer 2440. Opening 2462 extends to the top surface of lower contact pad 4, forming lower contact pad 2423. Referring now to FIG. 24M, in the present embodiment, focus waffle metal 2427 is formed over focusing structures 2424.

Another etch is performed as shown by step 2311 to complete the structure. Referring now to FIGS. 24M–24N, etch step 2311 is shown to extend opening 2461 and opening 2463 of FIGS. 24K–24L through sputtered molybdenum layer 2403 and evaporated molybdenum layer 2402, forming contact pad 2422 and removing that portion of sputtered molybdenum layer 2403 and evaporated molybdenum layer 2402 that overlie cone 2426.

In the process shown in FIGS. 23–24, dielectric layer 2440 and passivation layer 2441 protect upper electrodes 1810, preventing damage to upper electrode 1810 as typically occurs in prior art processes. By preventing damage to upper electrode 1810, upper electrode shorts and opens are prevented. In addition, because upper electrode 1810 is protected, column shorts in the frit seal region are eliminated. Also, because there is less exposed metal as compared with prior art processes, upper electrode to focus waffle shorts are decreased.

With reference now to FIGS. 25–26, yet another method for forming an electrode structure for a display device is shown. As shown by step 201 of FIG. 25, lower electrodes are formed over a substrate. A resistor layer and a dielectric layer are then deposited over the lower electrodes as shown by steps 202–203. A gate metal layer is deposited as shown by step 204, followed by the formation of upper electrodes as shown by step 205. Mask and etch step 206 forms a gate structure. A cavity is then etched as shown by step 2301.

## 22

A layer of sputtered molybdenum, a layer of evaporated molybdenum, and a second layer of sputtered molybdenum are then deposited as shown by steps 2302–2304. In one embodiment, steps 201–206 and 2301–2304 are identical to steps 201–206 and 2301–2304 of FIG. 23.

Referring now to step 2501 of FIG. 25, a mask and etch step is performed that selectively etches both sputtered molybdenum layers and the evaporated molybdenum layer. In the present embodiment, mask and etch step 2501 removes all of that portion of the sputtered molybdenum layers and the evaporated molybdenum layers that overlie the region where the upper electrode contact pad is to be formed. That is, in the present embodiment, structure 2431 shown in FIG. 24F is also removed during etch step 2501.

Referring to step 2502 of FIG. 25, a dielectric layer is deposited. In one embodiment, the dielectric layer is silicon dioxide.

Referring now to FIGS. 26A–26B, a substrate 1 is shown after steps 201–206, 2301–2304, and 2501–2502 of FIG. 25 have formed dielectric layer 2600, molybdenum layer 2401, evaporated molybdenum layer 2402, and sputtered molybdenum layer 2403 such that cone 2426 is formed. Also shown are gate metal layer 1811 and upper electrodes 1810 that overlie dielectric layer 6, resistor layer 5 and lower electrode 4.

Referring now to step 2503 of FIG. 25, mask and etch steps are performed. In one embodiment, mask and etch step 2503 includes three mask and etch steps, a first mask and etch step that produces the structure shown in FIGS. 26C–26D, a second mask and etch step that produces the structure shown in FIGS. 26E–26F and a third mask and etch step that produces the structure shown in FIGS. 26G–26H. Referring now to FIGS. 26G–26H, the third mask and etch step forms an opening that extends to lower electrode 4, forming contact pad 2643. In the present embodiment, first and second etches are dry etches and the third etch is a wet etch. However, the present invention is well adapted to the use of different mask and etch processes for producing the structure shown in FIGS. 26G–26H.

As shown in step 2504, focusing structures are formed. Referring to FIG. 26I, in the present embodiment, focus waffle metal 2627 is formed over focusing structures 2624. As shown by step 2505 of FIG. 25, an etch step is performed so as to further etch the remaining dielectric layer. In one embodiment, etch step 2504 uses a dry etch process. Referring now to FIGS. 26I–26J, step 2504 forms polyimide structures 2624 while step 2505 forms contact pad 2642.

Another etch is then performed as shown by step 2506 to complete the structure. In the present embodiment, as shown in FIGS. 26K–26L, etch step 2506 removes evaporated molybdenum layer 2553 and sputtered molybdenum layers 2552 and 2554.

Upper electrode 1810 is protected by dielectric layer 2600, preventing damage to upper electrode 1810 as typically occurs in prior art processes. By preventing damage to upper electrode 1810, upper electrode shorts and opens are prevented. In addition, because upper electrode 1810 is protected, column shorts in the frit seal region are eliminated. Also, because there is less exposed metal as compared with prior art processes, upper electrode to focus waffle shorts are decreased.

With reference now to FIGS. 27–28, yet another method for forming an electrode structure for a display device is shown. As shown by step 201 of FIG. 27, lower electrodes are formed over a substrate. A resistor layer and a dielectric layer are then deposited over the lower electrodes as shown

by steps 202–203. A gate metal layer is deposited as shown by step 204. Upper electrodes are then formed as shown by step 205. As shown by step 206, mask and etch steps are then performed to form a gate structure. Mask and etch steps are then performed as shown by step 2301 to form a cavity. In one embodiment, steps 201–206 and 2301 are identical to steps 201–206 and 2301 of FIG. 23.

Continuing with FIG. 27, a layer of evaporated chromium is then deposited as shown by step 2701, followed by the deposition of a layer of evaporated molybdenum as shown by step 2702. A dielectric layer is then deposited as shown by step 2703.

Referring to FIGS. 28A–28B, a substrate 1 is shown after steps 201–206 have formed lower electrodes 4, resistor layer 5, dielectric layer 6, gate metal structure 1811 and upper electrodes 1810. Etch step 2301 forms cavity 2425. Steps 2701–2703 result in the formation of evaporated chromium layer 2830, evaporated molybdenum layer 2831, and dielectric layer 2832.

Referring back to FIG. 27, as shown by step 2704, mask and etch steps are then performed. Referring now to FIGS. 28C–28D, step 2704 etches through dielectric layer 2832, molybdenum layer 2831, evaporated chromium layer 2830 and partially etches upper electrodes 1810.

Continuing with FIG. 27, as shown by step 2705, another etch step is performed that etches dielectric layer 6 and resistor layer 5, forming the structure shown in FIGS. 28E–28F. Step 2706 exposes a portion of lower electrode 4 so as to form contact pad 2823.

Continuing with FIG. 27, as shown by step 2706, the focusing structure is formed. Referring now to FIGS. 28G–H, focusing structure 2824 is shown to be formed. Referring now to FIG. 28G, in the present embodiment, focus waffle metal 2827 is formed over focusing structures 2824.

Continuing with FIG. 27, as shown by step 2707, an etch step is performed. Referring now to FIGS. 28I–28J, step 2707 is shown to remove dielectric layer 2832 and to partially remove a portion of dielectric layer 6.

Another etch is then performed as shown by step 2708 to complete the structure. FIGS. 28K–28L show the structure of FIGS. 28I–28J after step 2708 has been performed. In the present embodiment, etch step 2708 removes evaporated molybdenum layer 2831.

During process steps 2704–2708, upper electrode 1810 is protected by evaporated chromium layer 2830. This prevents damage to upper electrode 1810 as typically occurs in prior art processes. By preventing damage to upper electrode 1810, upper electrode shorts and opens are prevented. In addition, because upper electrode 1810 is protected, column shorts in the frit seal region are eliminated. Also, because there is less exposed metal as compared with prior art processes, column to focus waffle shorts are decreased.

The foregoing descriptions of specific embodiments of the present invention have been presented for purposes of illustration and description. They are not intended to be exhaustive or to limit the invention to the precise forms disclosed, and obviously many modifications and variations are possible in light of the above teaching. The embodiments were chosen and described in order to best explain the principles of the invention and its practical application, to thereby enable others skilled in the art to best utilize the invention and various embodiments with various modifications. It is intended that the scope of the invention be defined by the Claims appended hereto and their equivalents.

What is claimed is:

1. A method for forming an electrode structure of a display comprising:
  - a) depositing a layer of metal alloy over a backplate;
  - b) depositing a cladding layer over said layer of metal alloy such that said layer of cladding overlies said layer of metal alloy; and
  - c) etching said layer of metal alloy and said cladding layer using a wet etch process so as to form a plurality of electrodes, wherein said cladding layer comprises molybdenum and tungsten.
2. A method for forming an electrode structure of a display as recited in claim 1 wherein said metal alloy comprises a silver alloy.
3. A method for forming an electrode structure of a display as recited in claim 2 wherein said silver alloy comprises silver and palladium.
4. A method for forming an electrode structure of a display as recited in claim 3 wherein said silver alloy comprises from approximately 0.5 atomic percent palladium to approximately 2 atomic percent palladium.
5. A method for forming an electrode structure of a display as recited in claim 3 wherein said silver alloy further comprises titanium.
6. A method for forming an electrode structure of a display as recited in claim 5 wherein said silver alloy comprises up to approximately 2 atomic percent titanium.
7. A method for forming an electrode structure of a display as recited in claim 2 wherein said silver alloy further comprises from approximately 0.5 atomic percent copper to approximately 2 atomic percent copper.
8. A method for forming an electrode structure of a display as recited in claim 7 wherein said silver alloy comprises up to approximately 2 atomic percent titanium.
9. A method for forming an electrode structure of a display as recited in claim 1 wherein step a) and step b) are performed sequentially in a single sputtering tool.
10. A method for forming an electrode structure of a display as recited in claim 1 wherein said metal alloy comprises an aluminum alloy.
11. A method for forming an electrode structure of a display as recited in claim 10 wherein said aluminum alloy further comprises aluminum and neodymium.
12. A method for forming an electrode structure of a display as recited in claim 11 wherein said aluminum alloy comprises from approximately 0.5 atomic percent neodymium to approximately 6 atomic percent neodymium.
13. A method for forming an electrode structure of a display as recited in claim 11 wherein said metal alloy further comprises titanium.
14. A method for forming an electrode structure of a display as recited in claim 13 wherein said aluminum alloy comprises up to approximately 5 atomic percent titanium.
15. A method for forming an electrode structure of a display comprising:
  - a) depositing a first metal alloy layer over a backplate;
  - b) masking and etching said first metal alloy layer so as to form a plurality of first electrodes;
  - c) depositing a resistor layer over said plurality of first electrodes;
  - d) depositing a dielectric layer over said resistor layer;
  - e) depositing a second metal alloy layer over said dielectric layer;
  - f) masking and etching said second metal alloy layer so as to form a plurality of second electrodes;
  - g) depositing a layer of silicon nitride over said plurality of second electrodes, said layer of silicon nitride

## 25

adapted to protect said plurality of second electrodes during subsequent process steps.

16. A method for forming an electrode structure of a display as recited in claim 15 further comprising:

a1) disposing a cladding layer over said first metal alloy layer such that said layer of cladding overlies said first metal alloy layer.

17. The electrode structure of claim 16 wherein said cladding layer further comprises molybdenum and tungsten.

18. A method for forming an electrode structure of a display as recited in claim 15 wherein step b) further comprises:

b1) etching said first metal alloy layer and said layer of cladding sequentially in a single sputtering tool.

19. A method for forming an electrode structure of a display as recited in claim 15 further comprising:

a1) disposing a cladding layer over said second metal alloy layer such that said layer of cladding overlies said second metal alloy layer.

20. A method for forming an electrode structure of a display as recited in claim 15 wherein step f) further comprises:

f1) etching said second metal alloy layer and said layer of cladding sequentially in a single sputtering tool.

21. A method for forming an electrode structure of a flat panel display as recited in claim 15 wherein steps b) and f) are performed using an etchant that includes nitric acid and phosphoric acid and ascetic acid and water so as to form angled edges on each of said plurality of electrodes.

22. A method for forming an electrode structure of a flat panel display as recited in claim 15 wherein said first metal alloy layer and said second metal alloy layer comprise an aluminum alloy.

23. A method for forming an electrode structure of a flat panel display as recited in claim 15 wherein said first metal alloy layer and said second metal alloy layer comprise a silver alloy.

24. A method for forming an electrode structure of a display comprising:

- a) forming a plurality of first electrodes;
- b) depositing a resistor layer over said plurality of first electrodes;
- c) depositing a dielectric layer over said resistor layer;
- d) forming a plurality of second electrodes; and
- e) depositing a passivation layer over said plurality of second electrodes, said passivation layer adapted, to protect said plurality of second electrodes during subsequent process steps.

25. A method for forming an electrode structure as recited in claim 24 wherein said passivation layer further comprises a layer of silicon nitride.

26. A method for forming an electrode structure as recited in claim 25 further comprising the step of forming a gate structure, said gate structure disposed over said layer of silicon nitride.

27. A method for forming an electrode structure as recited in claim 25 further comprising the step of forming a gate structure, said gate structure disposed between said plurality of second electrodes and said layer of silicon nitride.

28. A method for forming an electrode structure as recited in claim 25 further comprising the step of forming a gate structure, said gate structure disposed between said dielectric layer and said plurality of second electrodes.

## 26

29. A method for forming an electrode structure as recited in claim 28 wherein said step of forming a gate structure further comprises the step of depositing a layer of gate metal, said layer of gate metal masked and etched prior to the deposition of said layer of silicon nitride.

30. A method for forming an electrode structure as recited in claim 28 wherein said step of forming a gate structure further comprises the step of depositing a layer of gate metal, said layer of gate metal masked and etched after the deposition of said layer of silicon nitride.

31. A method for forming an electrode structure as recited in claim 28 further comprising the step of forming a tantalum structure, said tantalum structure disposed between said gate structure and said plurality of second electrodes.

32. A method for forming an electrode structure as recited in claim 25 further comprising the step of depositing a dielectric layer prior to the step of depositing said layer of silicon nitride.

33. A method for forming an electrode structure of a display comprising:

- a) forming a plurality of first electrodes;
- b) depositing a resistor layer over said plurality of first electrodes;
- c) depositing a first dielectric layer over said resistor layer;
- d) forming a plurality of second electrodes; and
- e) depositing a second dielectric layer over said plurality of second electrodes, said second dielectric layer adapted to protect said plurality of second electrodes during subsequent process steps.

34. A method for forming an electrode structure as recited in claim 33 further comprising the step of depositing a first sputtered molybdenum layer over said plurality of second electrodes.

35. A method for forming an electrode structure as recited in claim 34 further comprising the step of depositing an evaporated molybdenum layer over said first sputtered molybdenum layer and depositing a second sputtered molybdenum layer over said evaporated molybdenum layer, said second dielectric layer disposed over said second layer of evaporated molybdenum.

36. A method for forming an electrode structure of a display comprising:

- a) forming a plurality of first electrodes;
- b) depositing a resistor layer over said plurality of first electrodes;
- c) depositing a first dielectric layer over said resistor layer;
- d) forming a plurality of second electrodes; and
- e) depositing a layer of evaporated chromium over said plurality of second electrodes, said layer of evaporated chromium adapted to protect said plurality of second electrodes during subsequent process steps.

37. A method for forming an electrode structure as recited in claim 36 further comprising the step of depositing an a second dielectric layer, said second dielectric layer disposed over said layer of evaporated chromium.

38. A method for forming an electrode structure as recited in claim 37 further comprising the step of depositing an evaporated molybdenum layer over said layer of evaporated chromium, said second dielectric layer disposed over said layer of evaporated molybdenum.